

Feb. 5, 1963

A. T. CAPE ET AL

3,076,704

IRON-BASE ALLOYS

Filed March 14, 1961



Fig. 1



Fig. 2

INVENTORS.

ARTHUR T. CAPE  
BY HERBERT CLARKE

*Ister & Ornstein*

ATTORNEYS

# United States Patent Office

3,076,704  
Patented Feb. 5, 1963

1

3,076,704

## IRON-BASE ALLOYS

Arthur T. Cape, Monterey, Calif., and Herbert Clarke, Hillsdale, N.J., assignors to Coast Metals, Inc., Little Ferry, N.J., a corporation of Delaware

Filed Mar. 14, 1961, Ser. No. 95,608

4 Claims. (Cl. 75—128)

This invention relates generally to iron-base alloys, but has reference more particularly to an iron-base alloy which is especially useful for manufacture into roller mill guides for steel mills.

Roller mill guides for steel mills, of which a typical example is illustrated in the accompanying drawing, in which FIG. 1 is an end elevational view of such a guide, and FIG. 2 is a cross-sectional view, taken on the line 2—2 of FIG. 1, have portions or areas which are of varying cross-section, so that it is important that the material which is used for manufacture into such guides have excellent toughness, heat-resistance, resistance to impact, and relative freedom from susceptibility to "heat checking," i.e., the development of fine cracks on the surface of the guides.

We have found that an iron-base alloy which has all of these properties has a composition which falls within the following ranges:

|            | Percent  |
|------------|----------|
| Carbon     | 1 to 3   |
| Chromium   | 15 to 20 |
| Nickel     | 4 to 8   |
| Cobalt     | 28 to 35 |
| Tungsten   | Up to 3  |
| Molybdenum | Up to 3  |
| Iron       | Balance  |

A preferred composition is one containing about 2% carbon, about 18% chromium, about 6% nickel, about 30% cobalt, about 2½% tungsten, about 2½% molybdenum, and about 39% iron.

The relatively high cobalt content produces an alloy having extreme toughness, and renders the alloy virtually immune to "heat-checking."

If the tungsten and molybdenum were not present in the alloy, the alloy would have increased toughness, but the small amounts of tungsten and molybdenum which

2

are incorporated in the alloy increase its heat-resistance, at the expense of some resistance to impact, and the net result is an alloy which is peculiarly satisfactory for manufacture into roller guides.

5 The alloy is more austenitic than alloys previously used for this purpose, and roller guides made from the alloy have virtually twice the life of guides presently made from such previously used alloys.

The alloy may contain one or more residual or trace elements, such as silicon, manganese, sulphur, phosphorus, etc., but the total of such elements should not exceed 3%. It is to be understood, therefore, that the phrase "substantially all iron," as used in the claims, is to be construed as inclusive of such a combined total of residual or trace elements.

10 It will be understood that various changes in the aforesaid alloys may be made, within the scope of the appended claims.

Having thus described our invention, we claim:

20 1. An alloy which is especially useful for manufacture into roller mill guides for steel mills, said alloy consisting of from 1 to 3% carbon, 15 to 20% chromium, 4 to 8% nickel, 28 to 35% cobalt, tungsten in appreciable amounts up to 3%, molybdenum in appreciable amounts up to 3%, and the balance substantially all iron.

25 2. An alloy which is especially useful for manufacture into roller mill guides for steel mills, said alloy consisting of about 2% carbon, about 18% chromium, about 6% nickel, about 30% cobalt, about 2½% tungsten, about 2½% molybdenum, and about 39% iron.

30 3. A roller mill guide for steel mills, said guide comprising an alloy consisting of from 1 to 3% carbon, 15 to 20% chromium, 4 to 8% nickel, 28 to 35% cobalt, tungsten and molybdenum each in an appreciable amount up to 3%, and the balance substantially all iron.

35 4. A roller mill guide for steel mills, said guide comprising an alloy consisting of about 2% carbon, about 18% chromium, about 6% nickel, about 30% cobalt, about 2½% tungsten, about 2½% molybdenum, and about 39% iron.

## References Cited in the file of this patent

### FOREIGN PATENTS

716,277 France Dec. 17, 1931